

## UNITED STATES PATENT OFFICE

ROBERT G. CAMPBELL, OF NEW YORK MILLS, NEW YORK

## SPUN CELLULOSE AND VISCOSA PRODUCTS

No Drawing.

Application filed August 11, 1926. Serial No. 128,702.

This invention relates, primarily, to spun cellulose and viscose products; it has more especial reference to a filament, element or yarn adapted for textile purposes; and it essentially involves such an element or filament as a unique product resulting from certain treatment, including spinning.

Rayon (so-called), artificial silk (as it is also designated), and similar cellulose and viscose filaments are now extensively utilized in the textile art for making fabrics, etc. Because of certain recognized commercial objections to and inherent defects in these filaments, their use has, to a certain extent and for that reason, been somewhat limited. For instance, the cellulose filament, when subjected to wetting, loses considerable of its tensile strength and, as a result, fabric manufactured therefrom has proved more or less unsatisfactory. In other words, its wet-strength is materially less than its dry-strength. Much experimentation has, as a result, been conducted in an attempt to cure this serious defect; but, so far as I am aware, no successful treatment has, before my invention, been proposed. To compensate for the inherent weakness of the element, it has been rather common practice to combine therewith in knitting or weaving other materials, such as silk, wool, etc. Another objection to rayon and similar products is that it is quite harsh to the feel and, for that reason, does not always favorably compare with genuine silk when knit or woven into fabric for certain types of wearing apparel. Still another objection to this product is its relative unworkability in certain machines, requiring certain incidental treatment to adapt it therefor.

It is the object of the present invention to provide a product which has none of these objections. In other words, I have developed a cellulose-element which possesses a satisfactory degree of strength and durability, even after being wetted; for commercial purposes; it is relatively soft; and it is readily workable in knitting and weaving machines.

My inventive-concept may, therefore, be defined as a spun rayon textile element including cellulose only. In other words, by

subjecting rayon and the like to a spinning operation, I am enabled to produce a unique product which marks a distinct advance in the art, as demonstrated by practical tests and observations.

Usually, rayon, etc., comes to the trade in relatively long, untwisted filaments or strands and of various diametral sizes and characteristics; and it is usual practice to run these strands through knitting and weaving machines in the condition they are in when they come from their manufacturer: It is a feature of my concept to treat these strands in a manner that changes certain of their characteristics whereby they are greatly improved and rendered more adaptable in the knitting and weaving operations and more serviceable in use. In the first place, these strands or threads (as I shall hereinafter call them for convenience), preferably while dry, are cut into relatively short lengths. In other words, they are subjected to an operation whereby they are reduced to lengths, say, of one and one-half inches. If these elements, so cut, are in readily separable and clean condition, they are subjected, successively, to the steps of picking and carding to condition them for spinning, all as more particularly explained in my companion application Serial No. 128,703, filed August 11, 1926, and entitled "Method of producing spun rayon elements".

It will be understood, therefore, that the mass of threads furnished by rayon manufacturers is, under my concept, cut into predetermined short lengths and, then, spun to effect an interlacing of their component parts whereby an element or yarn results which possesses, to a recognizable degree, tensile strength and softness that improve its qualities and properties for fabric purposes. In other words, the resultant product of my method of spinning together cut rayon filament shows, when wet, a far less loss of tensile strength than the original filament when wetted. The compounding of the cut filament sections does not, of course, lend any greater wet-strength to the individual filaments, but it does make the element com-

55

65

75

80

85

90

95

100

pounded of these individual filaments of appreciably greater strength.

I am not now prepared to explain why the spinning operation so appreciably adds to the strength of the element; but tests have proved that this characteristic is undeniably introduced thereinto, such that fabric knit or woven therefrom, even when wetted, does not indicate the weakness which is, as aforementioned, invariably present in rayon, etc., after being moistened. The softness which the spun element develops is probably due to breaking of the long filaments of commerce into short lengths so that, when these fibers are brought into combinative association by spinning, the resultant element will possess greater relative flexibility and will likewise possess greater softness.

It is to be understood that rayon, or artificial silk, as produced by its manufacturers, comprises a predetermined number of filaments combined to constitute a strand or thread of a certain number of deniers. For instance, the customary sized rayon filament used in knitting hosiery and underwear is 150 deniers, which means that a thread of 150 deniers would be composed of twenty-five six-denier filaments. These filaments are not twisted or spun together in any technical sense.

The desideratum, under my concept, is so to combine the small-dimensioned filaments, pre-cut to relatively short lengths, that they shall, in the ultimate product, have their components combinatively associated. This is effected by the spinning operation.

I am aware of the fact that it has heretofore been proposed to cut artificial filaments into relatively long lengths—four inches or more—and combine them under the so-called "worsted" or "schappe" spinning processes. The thread resulting from these practices, however, is quite different in structure from the element produced by the procedure followed by me and wherein there is an intimate combination effected between the several filaments by imparting to the element a substantial twist.

I am also aware of the fact that it has heretofore been proposed to cut artificial filaments into spinnable lengths and then, following an intermediate operation, spin the same. But my inventive-concept is distinguishable therefrom in that, in that instance, cotton is mixed with the artificial filament and, then, this mass is subjected to the action of a lapper-machine, after which the cotton is combed out. The combing operation, I have found in practice, is detrimental to satisfactory spinning; and, besides, the introduction of the cotton to and its removal from the mass of cut filaments involves an expensive and unnecessary operation. The resultant of my procedure is an uncombed spun rayon textile element, unaffected by hav-

ing been associated with any other fiber during the operation of making it spinnable.

As the result of experiments and tests, it has been found that, by cutting the fine rayon filaments in lengths of approximately one and a quarter to two inches, and spinning these together, as already explained, the new type of textile element is produced, with all of the desirable characteristics of the original filament retained, and with certain additional and desirable characteristics developed therein.

Where I have herein used the term "relatively short lengths" and similar expressions, it is to be understood that I mean these to comprehend and embrace sections from one and a quarter to two inches, approximately. Experiments indicate that lengths less than one and a quarter inches do not permit of the necessary interlacing of the individual fibers to provide the required strength of the element. On the other hand, sections of substantially greater length than two inches do not work well in the different operations utilized to produce my product.

Where I have herein used the expression "wet strength" or equivalent terms, I mean thereby the strength of the mass when saturated or substantially moistened.

It is to be understood that any loss of luster resulting to the product from the cutting and spinning operations referred to is not detrimental; but, if it be desirable to restore such luster, any appropriate gloss-producing operation may be employed. It has been discovered that the element may be subjected to moistening and stretching (as effected in accordance with the procedure outlined in the companion application of W. M. Sternberg, filed August 27, 1926, Serial No. 131,966) for this purpose.

In using the expressions "soft", "softness" and like words, I refer to the condition imparted to the product by the steps recited, and which terms, necessarily relative, imply that such product has that characteristic as compared with the original commercial rayon filament.

Where I have herein employed the expressions "rayon", "artificial silk" and similar terms, it is to be understood that they and equivalent designations for the material employed in connection with my invention, shall comprehend and include any thread, thread-formation, filament or fiber, in the nature of a more or less lustrous textile element converted from cellulose (whether it be obtained from wood, cotton or any other vegetable material) by means of chemical and mechanical processes, and whether such basic mass be known as cellulose or viscose.

Where, in the claims, I refer to a rayon-element, I mean to designate the commercial product of rayon manufacturers as used by the knitter or weaver, which element is regu-

larly composed of a plurality of fine rayon filaments arranged in substantial parallelism to provide a thread or yarn-forming group.

Where I have herein used the terms "spinning", "spun", etc., as involving essential steps in my procedure, I wish it to be understood that these terms comprehend that type of textile-yarn manufacturing process which embodies, as its essence, the appreciable and substantial drawing and twisting of the original sliver of material into the finished yarn or thread. These terms are not intended to include so-called "schappe spinning".

15 What I claim is:

1. A rayon textile element comprising a multiplicity of relatively short cellulose filament sections of substantially equal length spun together without other material.

20 2. A rayon textile element comprising solely a multiplicity of relatively short-length uncombed filaments of cellulose spun directly together.

25 3. A rayon textile element comprising a multiplicity of relatively short uncombed filament sections composed solely of cellulose, said filament sections being of substantially uniform length and spun together without other material.

30 In testimony whereof, I affix my signature.  
ROBERT G. CAMPBELL.

35

40

45

50

55

60

65